

3,203,999

## FLUORINATED CHEMICAL COMPOUND

David Milton Gardner, North Wales, Pa., Robert Edward Oesterling, Silver Spring, Md., and Murray Hauptschein, Glenside, Pa., assignors to Pennsalt Chemicals Corporation, Philadelphia, Pa., a corporation of Pennsylvania  
No Drawing. Filed June 28, 1962, Ser. No. 207,157  
1 Claim. (Cl. 260—633)

This invention relates to the new compound 2,2-difluoro-2-nitroethanol, particularly useful as a stable monopropellant for rocket propulsion.

The desired characteristics for a high performance monopropellant are high specific impulse, high thermal stability, good storage stability and ease of handling. The specific impulse value is a measure of the total thrust available from a given weight of propellant. (See Rocket Propulsion Elements, George P. Sutton, John Wiley & Sons, Inc., New York, 1949, particularly pages 18 and 19.) High thermal stability is important in a liquid monopropellant since it is desirable to use the monopropellant itself as a coolant in a regeneratively cooled rocket engine system. In such applications, the monopropellant may be heated, e.g., to average temperatures of 300° F. and higher, and should be able to withstand such temperatures without thermal decomposition. Good storage stability is obviously desirable, and it is also desirable that the monopropellant be relatively non-volatile and non-corrosive in character so that it can be handled without special precautions.

According to the present invention, it has been found that the new compound 2,2-difluoro-2-nitroethanol,  $\text{CF}_2\text{NO}_2\text{CH}_2\text{OH}$ , possesses all the above desired properties to a high degree. It has a high specific impulse of 241 pounds per second per pound. It shows no significant decomposition when heated for long periods at a temperature of about 400° F. It is a relatively non-volatile liquid having excellent storage stability. It is essentially non-corrosive with respect to all ordinary materials of construction such as metals and glass, many plastics and thus can be stored and handled without special precautions.

The desirable properties of  $\text{CF}_2\text{NO}_2\text{CH}_2\text{OH}$  as a monopropellant are apparent when this compound is compared on the basis of specific impulse, thermal stability, storage stability and ease of handling with other typical monopropellants. In Table I, such a comparison is shown between  $\text{CF}_2\text{NO}_2\text{CH}_2\text{OH}$  and four well-known monopropellants.

TABLE I

|                                    | Specific impulse, lb./sec./lb. | Thermal stability                                  | Storage stability                                            | Ease of handling                                                                                       |
|------------------------------------|--------------------------------|----------------------------------------------------|--------------------------------------------------------------|--------------------------------------------------------------------------------------------------------|
| 2,2-difluoro-2-nitroethane-----    | 241                            | Stable on heating for 8 hrs. at 200° C. (392° F.). | Stable indefinitely under normal storage conditions.         | Not highly flammable. Stores as a liquid at normal pressure and temperature in conventional container. |
| Amine nitrates in nitric acid----- | 256                            | Decomposes above 250° F.                           | Stable if stored in acid proof containers.                   | Highly corrosive, strong oxidizing agent.                                                              |
| Hydrazine-----                     | 221                            | Unstable over 200° F.                              | Stable only when stored under rigidly controlled conditions. | Moderately toxic, highly inflammable, subject to catalytic violent decomposition.                      |
| Ethylene oxide-----                | 198                            | do-----                                            | Must be stabilized to prevent polymerization.                | Must be stored under pressure, highly inflammable. May polymerize violently.                           |
| Hydrogen peroxide-----             | 155                            | do-----                                            | Slow, spontaneous decomposition on storage.                  | Severe explosion hazard. Ignites most combustible materials on contact.                                |

The ideal specific impulse (in pounds of thrust delivered at a propellant flow rate of one pound per second) was determined for conditions of shifting equilibrium during expansion and for a pressure in the combustion chamber

and exhaust, respectively, of 1000 p.s.i. and 14.7 p.s.i. The determination was made according to the method described in "Thermodynamics of High Temperature Gas Mixtures and Application to Combustion Problems," by John S. Gordon, PB 133980, U.S. Govt. Research Reports, November 14, 1958.

$\text{CF}_2\text{NO}_2\text{CH}_2\text{OH}$  may be prepared by the addition of dinitrogen tetroxide to 1,1-difluoroethylene ( $\text{CH}_2=\text{CF}_2$ ) to form a nitro-nitrite addition product which may be converted by alkaline hydrolysis to the nitroalcohol. The reaction is believed to proceed as follows:



The reaction is desirably carried out in the presence of a solvent which is unreactive to  $\text{N}_2\text{O}_4$  under the reaction conditions. Without a solvent, the addition reaction is difficult to control, and explosion may occur. Preferred are the halogenated solvents, particularly the chlorinated or chlorofluorinated solvents such as chloroform, methylene chloride ( $\text{CH}_2\text{Cl}_2$ ), carbon tetrachloride, trichlorotrifluoroethane, dichlorotetrafluoroethane, etc. The amount of solvent is not critical and generally may be used in an amount ranging from 100 to 1000 milliliters per mole of olefin. Desirably the reaction is carried out under substantially anhydrous conditions to avoid reactions between  $\text{N}_2\text{O}_4$  and water and the possibility of other side reactions.

Preferably the reaction is carried out under moderate pressures of, e.g., 100 to 2,000 lbs./in.<sup>2</sup> and at moderate temperatures of, e.g., 20° C. to 100° C. Approximately equimolar amounts of 1,1-difluoroethylene and dinitrogen tetroxide are usually employed. Following the formation of the dinitrogen tetroxide addition product by the above procedure, the addition product is hydrolyzed, preferably using a weak aqueous alkaline solution, such as a sodium bicarbonate solution, and the hydrolysis product  $\text{CF}_2\text{NO}_2\text{CH}_2\text{OH}$  then isolated by decantation of the organic portion and extraction with ether or other suitable solvent of the aqueous portion, and vacuum distillation.

The following example illustrates the preparation of  $\text{CF}_2\text{NO}_2\text{CH}_2\text{OH}$  by the above procedure.

## Example 1

A stainless steel autoclave of 1 liter capacity is charged with 110 grams of dinitrogen tetroxide dissolved in 500 grams of  $\text{CCl}_2\text{CCl}_2\text{F}$  at 0° C. after which 150 grams of  $\text{CH}_2=\text{CF}_2$  is introduced by vacuum transfer with the 50 autoclave cooled in liquid nitrogen. The sealed auto-

clave is then placed on a mechanical shaker and allowed to warm to room temperature. An exothermic reaction ensues causing a temperature increase to about 90° C. and a pressure increase to 900 lbs./in.<sup>2</sup>. Agitation is con-

tinued for 8 hours during which time the autoclave cools to 30° C. and the pressure decreases to 500 lbs./in.<sup>2</sup>.

The autoclave is vented and the liquid contents poured into an equal volume of water to which is added, with stirring, a sodium bicarbonate solution until neutralized. The organic layer is separated and dried over anhydrous magnesium sulfate and after removal of  $\text{CClF}_2\text{CCl}_2\text{F}$  by distillation 10 grams of a pale yellow oil is obtained the middle cut of which, boiling at 47° C. at about 12 mm. Hg, is the nitro alcohol  $\text{CF}_2\text{NO}_2\text{CH}_2\text{OH}$ . The infrared spectrum of this compound shows the characteristic OH band at  $2.99\mu$  (bonded); the characteristic  $\text{NO}_2$  band at  $6.3\mu$  and carbon-fluorine stretching vibrations, at 8–10 $\mu$ . The aqueous layer is acidified and then extracted three times with diethyl ether, the ether solution dried and evaporated to give 25 grams of a red oil, which on vacuum distillation, is shown to consist of mostly  $\text{CF}_2\text{NO}_2\text{CH}_2\text{OH}$ . A middle cut boils at 63° C. at about 20 mm. Hg. The N-phenyl carbamate ester of the 2,2-difluoro-2-nitroethanol is prepared with phenyl isocyanate using triethylamine as a catalyst. Recrystallization of the ester



from a light petroleum ether-benzene mixture and vacuum sublimation gives colorless needles melting at 42–43° C.

*Analysis.*—Calculated for  $\text{C}_9\text{H}_8\text{F}_2\text{N}_2\text{O}_4$ : C, 43.91; H, 3.27; N, 11.4. Found: C, 44.15; H, 3.14; N, 11.8.

The compound of the invention may also be prepared by the reduction of difluoronitroacetic acid



10 The precursor compound  $\text{NO}_2\text{CF}_2\text{COOH}$  can be readily prepared by the reaction of  $\text{N}_2\text{O}_4$  with tetrafluoroethylene followed by hydrolysis of the addition product in accordance with the following:



Reduction of the acid may be accomplished in various ways such as with diborane formed in situ by the reaction of boron trifluoride etherate with sodium borohydride.

We claim:

The compound 2,2-difluoro-2-nitroethanol.

No references cited.

LEON ZITVER, *Primary Examiner.*

LEON D. ROSDOL, *Examiner.*